

March 8, 1932.

E. LIONNE

1,848,732

SHOE STIFFENER AND METHOD OF MAKING IT

Filed Nov. 29, 1929



Fig. 1.



Fig. 2.

Inventor

Ernest LIONNE

*W. Greenwood*  
Atty

## UNITED STATES PATENT OFFICE

ERNEST LIONNE, OF NAHANT, MASSACHUSETTS

## SHOE STIFFENER AND METHOD OF MAKING IT

Application filed November 29, 1929. Serial No. 410,354.

This invention relates to stiffeners for boots and shoes and to sheet material from which the stiffeners can be made.

In my copending application Serial No. 308,082, filed September 24, 1928, I have described a sheet material and a stiffener made therefrom wherein the sheet material is composed of fibres, some of which are soluble in a suitable solvent and are capable of being converted from a fibrous to a colloidal or gelatinous form which when the solvent has evaporated, form a stiff hard film in which the remaining or insoluble fibres of the sheet are bound. The sheet, specifically, is composed of insoluble fibres such as textile fibres, wood fibres, and generally the usual paper making fibres, and combined with soluble fibres such as pyroxylene, cellulose acetate, or other suitable cellulose esters. The sheet is made by intermixing the insoluble and soluble fibres in a beater and forming the sheet by customary paper making methods.

The stiffener made from such sheet had many advantages over prior stiffeners. I have found, however, that I can improve upon this type of stiffener. Pyroxylene and other fibres of this general type are harsh and brittle and do not felt with themselves and with the insoluble paper making fibres as well as is desired, so that the resulting sheet is fragile and is difficult to handle without rupturing it when it is wet with solvent unless more care is given to the manufacture of the sheet than is desired. Furthermore, the dispersion of the soluble fibres in the sheet is not uniform and the sheet contains spots made of bunched soluble fibres, which is not desirable.

I have found that I can obtain a better sheet and stiffener and one having more tightly felted fibres, greater mechanical strength, and uniformly dispersed soluble material, if instead of making the sheet with a mixture of the soluble and insoluble fibres, I first comminute the soluble fibres and destroy the fibrous nature thereof, as by pulsing them into extremely fine particles, and thoroughly intermix the comminuted particles and the insoluble paper making fibres and form a sheet from such mixture. This

constitutes an object of the present invention.

In carrying out the invention, the pyroxylene or other soluble cellulose ester fibres alone are introduced, with the addition of water, into a paper beater and the beater is operated for so long as is necessary to comminute the fibres or to obtain the requisite degree of fineness, and, preferably, to pulp them into extremely fine particles which may be a matter of hours. The beater should be operated long enough to destroy completely the fibrous structure and reduce the fibres to the condition of a finely ground pulp, the degree of fineness of the comminuted material being at least such that the material can not be felt with the insoluble fibres of the paper making stock. After the soluble material has been comminuted, it is mixed with any usual or desired paper making fibres in the beater and the beater is operated until a thorough dispersion of the comminuted soluble particles throughout the mass of paper making stock is effected, this dispersion being effected without difficulty since the soluble particles are fine as compared with the size of the paper making fibres and have approximately the same density as the fibres. The paper making fibres may be anything usual in the art as rag stock, wood fibres, and the like. The mixture of comminuted material and paper stock is then flowed from the stuff box of the usual paper making machine onto the paper making wire in a Fourdrinier or cylinder machine, or the paper can be laid in any desired manner. The insoluble or paper making fibres on the wire become felted together in the usual manner. The comminuted soluble material occupies the voids between the insoluble fibres. The sheet thus formed can be dried and calendered as is usual in paper making. Preferably, however, the temperature of drying should not be so great as to decompose the particles of comminuted material. The calendering should be light enough to provide a paper sheet which is porous so that it can be penetrated rapidly by a suitable solvent for the comminuted material.

Since the comminuted soluble material oc-

55

60

65

70

75

80

85

90

95

100

copies the voids between the paper making fibres, these fibres can felt together without hindrance and without any unusual attention being paid to the formation of the sheet. The sheet can thus be made sufficient mechanically strong so that the stiffener cut therefrom can withstand the usual operations without becoming torn, since there is no opposition to the felting or interlacing of the insoluble paper making fibres. The soluble comminuted material is uniformly dispersed throughout the sheet and does not collect in isolated spots, as with the sheet formed with soluble fibres, and the material occupies the voids between the insoluble felted fibres and it is retained therein by the interlacing of such fibres. When the sheet, or a stiffener cut therefrom, is treated with a solvent for the comminuted material, which solvent can be any well known solvent as acetone, wood alcohol, and the like, the comminuted particles are converted to a colloidal or gelatinous form, which, especially when assisted by the pressure of lasting the shoe with a stiffener therein, spreads throughout the stiffener and in between and over the insoluble fibres thereof and unites when the solvent has evaporated to form a stiff uniform film which is integral and is dispersed uniformly throughout the body of the stiffener and which encloses and bonds together the insoluble fibres and retains the stiffener in the shape imparted to it by the last.

The proportion of comminuted material to insoluble fibres can be varied within wide limits. For a relatively stiff stiffener, equal parts of comminuted material and insoluble fibres can be used. Where a stiffener having less stiffness is satisfactory, the amount of comminuted soluble material can be reduced. For convenience and economy, I employ a material consisting of comminuted nitro-cellulose fibre but not do not necessarily limit myself to this material as other esters of cellulose such as cellulose acetate, butyl cellulose and the like, can be employed, or other material formed from film-forming fibres which are soluble in a suitable solvent and, preferably, are insoluble in water, so that the stiffener will not lose its shape when the shoe in which it is built becomes wet.

I have found that the use of comminuted material prepared from soluble fibres has a number of advantages over a soluble material which exists in another form, as celluloid in a granular form.

My comminuted material has approximately the density of the usual paper making fibres so that it can be dispersed uniformly throughout the paper stock and kept in suspension therein and thus can produce a uniform paper sheet. By reason of its ability to remain in suspension, but a small amount of the material is lost through the paper making wire. A granular celluloid is ma-

terially heavier than the paper making fibres and does not readily remain in suspension in and in dispersed condition throughout the paper stock so that the resulting sheet is not readily made uniform and a considerable quantity of the granules is lost through the paper making wire. My comminuted material hydrates to some degree during the heating process so that, in the finished sheet, the particles adhere together and to the adjacent fibres, thereby preventing loss of material through the wire and making a stronger sheet than a granular celluloid which does not hydrate so that its particles have no affinity for themselves or for the paper making fibres. 70

The dry sheet made from my material does not lose comminuted material when the sheet is wrapped, while a sheet having granular celluloid will have its granular particles shaken out. 85

In the drawings, Fig. 1 is a plan view of a shoe stiffener embodying the invention and Fig. 2 is an enlarged section of the material composing the stiffener, wherein 10 represents the insoluble interlaced or felted fibres and 12 the comminuted soluble particles made from soluble fibres and which occupy the voids between the felted insoluble fibres but are not interlaced therewith. 95

I claim:

1. A shoe stiffener containing interlaced insoluble fibres and comminuted particles of soluble fibrous material contained in the voids between the insoluble fibres. 100
2. A paper sheet composed of felted insoluble fibres and comminuted particles of soluble fibrous material contained in the voids between the felted fibres. 105
3. A shoe stiffener containing interlaced insoluble fibres and comminuted particles of a fibrous cellulose ester contained in the voids between the insoluble fibres. 110
4. A shoe stiffener containing interlaced insoluble fibres and comminuted particles of pyroxyline fibres contained in the voids between the insoluble fibres. 115
5. A paper sheet composed of felted insoluble fibres and comminuted particles of a fibrous cellulose ester contained in the voids between the felted fibres. 120
6. A paper sheet composed of felted insoluble fibres and comminuted particles of pyroxyline fibres contained in the voids between the felted fibres. 125
7. A paper sheet composed of felted insoluble fibres and comminuted particles of a soluble hydratable fibrous material contained in the voids between the felted fibres. 130
8. A paper sheet composed of felted insoluble fibres and comminuted particles of a soluble fibrous material contained in the voids between and free from felting relation with the felted fibres.
9. A paper sheet composed of felted in-

soluble fibres and comminuted particles of soluble fibrous material contained in the voids between the felted fibres, the particles having such a degree of fineness that they are incapable of felting with the felted insoluble fibres.

5 10. A paper sheet composed of felted insoluble fibers and comminuted particles of soluble fibrous material contained in the voids between the felted fibres, the particles having such a degree of fineness that they are incapable of felting with the felted insoluble fibres, and having approximately the density of the insoluble fibres.

15 11. A shoe stiffener containing felted insoluble fibres and unfelted pyroxline.

12. A paper sheet composed of felted insoluble fibres and comminuted particles of soluble fibrous material contained in the voids 20 between the felted fibres, the soluble particles having approximately the density of the insoluble fibres.

13. The method of making a paper sheet which consists in beating soluble fibres in a 25 paper beater until the fibres are comminuted, mixing the comminuted fibrous material with insoluble paper making fibres, and forming a sheet from such mixture.

14. The method of making a paper sheet 30 which consists in forming a paper sheet from a mixture of insoluble paper making fibres and soluble fibres which have been comminuted to such a degree of fineness that they cannot felt with the paper making fibres.

35 15. A shoe stiffener containing interlaced insoluble fibres and comminuted film forming particles of a soluble fibrous material contained in the voids between the insoluble fibres.

40 16. A shoe stiffener containing interlaced insoluble fibres and comminuted film-forming particles of a soluble fibrous material which is insoluble in water contained in the voids between the insoluble fibres.

45 In testimony whereof, I have signed my name to this specification.

ERNEST LIONNE.